

R. G. COATES,  
PROCESS FOR CASTING STEEL INGOTS,  
APPLICATION FILED AUG. 20, 1917.

1,327,987.

Patented Jan. 13, 1920.

FIG. 1.



FIG. 2.



FIG. 3.

WITNESSES.

*Nelson W. Bell*  
*Regina K. Schuster.*

INVENTOR.

*Ray G. Coates*

# UNITED STATES PATENT OFFICE.

RAY G. COATES, OF PASADENA, CALIFORNIA, ASSIGNOR, BY DIRECT AND MESNE ASSIGNMENTS, TO VALLEY MOULD AND IRON CORPORATION, OF NEW YORK, N. Y., A CORPORATION OF NEW YORK.

## PROCESS FOR CASTING STEEL INGOTS.

1,327,987.

Specification of Letters Patent. Patented Jan. 13, 1920.

Application filed August 20, 1917. Serial No. 187,166.

To all whom it may concern:

Be it known that I, RAY G. COATES, a citizen of the United States, residing at Pasadena, in the county of Los Angeles and State 5 of California, have invented a new and useful Improvement in Processes for Casting Steel Ingots, of which the following is a specification.

The customary method of casting steel 10 ingots for rolling is to pour the metal into iron chills, usually set vertically. Due to well known reasons a "pipe" forms in the central upper part of the ingot; a tendency to segregation of certain of the constituents 15 occurs in the region of the pipe; the gases discharged from the molten metal in solidifying have to travel from the lower part of the mold to the upper part to be discharged at the surface and it results that a large 20 part of these gases fail to reach the surface. The various methods of heating the upper part of the ingot so as to keep feeding the pipe with fluid metal have been but partially 25 successful in preventing the pipe, the segregation of constituents, the accumulation of gases in a part of the ingot, and the formation of "scrap". With all of the present 30 precautions rails rolled from the two ends of the ingot have different characteristics in some degree.

Figure 1 illustrates one form of mold in which my process may be carried out. Fig. 2 illustrates a different type of chill mold. Fig. 3 is a cross-sectional view showing a 35 hot cover over the mold and illustrating in dotted lines the formation of crystallization zones.

The principal object of my invention is to render the various cross sections of the 40 ingot of a more nearly average chemical and physical constitution than now obtains, and to do away with the pipe to such an extent that cropping of the ingot will not be necessary for either physical or chemical reasons. Incidental advantages will appear 45 later.

Another object of the present invention is the method of forming steel ingots by casting the ingots in a shallow mold and controlling the temperature over the surface of the molten steel by means of a hot gaseous envelop through which gases expelled from the steel may freely escape, and controlling the temperature in such manner that solidi- 50

fication of the ingot travels gradually from 55 the bottom thereof to the top surface thereof.

A further object of the present invention is the production of an article of manufacture comprising an ingot of steel wherein 60 the zones of solidification extend lengthwise of the ingot and are in cupped form with the long side of the ingot comprising the mouth of the cups and with the cups of decreasing depth when measured on the mid 65 cross-section plane at right angles to the said long side.

These results I accomplish by casting the metal in chills in which the axis of the ingot is horizontal and in which a long side, instead of an end, of the ingot is open, and by maintaining the metal hot on this long side by the application of heat while the metal of the ingot is crystallizing from the bottom and sides of the chill. When cast 70 in this position the gases discharged from the crystallizing metal in order to reach the surface have to travel through the fluid metal an average distance of only half the thickness of the ingot instead of an average 75 distance of half the length of the ingot as when cast vertically. Preferably the application of heat to the metal of the ingot is accomplished through the use of a heated atmosphere maintained over the surface of 80 the molten steel, in such manner that the heated atmosphere or gaseous envelop does not interfere with the free emission of gases 85 from the molten steel as it cools. This gaseous envelop or atmosphere may be secured by means of a heat-radiating substance or otherwise. The flotation tendency of the gas bubbles is greater since the head of metal is less than in the vertically 90 cast ingot and the bubbles are therefore less compressed consequently they more quickly 95 reach the still fluid surface and are released from the ingot. Since the horizontal cross section of the metal is larger than in the vertically cast ingot the gases do not travel 100 toward the surface in the same paths and it results that such as are not discharged do not gather into large accumulations near the top of the ingot. The tendency to form a pipe is very small since there are only three 105 chilled sides cross sectionally of the ingot, thus allowing the relatively large area of the top to feed the contraction of the metal

below, there being more top surface of the ingot, than when cast vertically, for heat absorption to keep the metal fluid until it crystallizes from the bottom and sides of the chill. The pipe degenerates into a slight "sinking in" of the top surface of the ingot and this will roll out in the first pass in rolling. Whatever variation in the chemical constitution of the ingot may occur, due to gravity and the direction of cooling toward the last remaining fluid surface such variation will still result in a homogeneous condition longitudinally of the ingot since each cross section will be approximately alike. Thus the rolled product from both ends of the ingot will be similar. This is a matter of great importance in the case of rails and long heavy beams.

In the drawings, which are diagrammatical, Fig. 1 represents a two part chill. This amounts to a very squat form of the common chill with the further difference that one of the interior horizontal dimensions is increased to the length of ingot desired. To release the ingot the chill, 1, is lifted from its stool, 2, in the usual way, since the draft of the chill is toward the bottom of the ingot. Fig. 2 represents a one piece chill, the draft here being toward the top of the chill. The ingot is released by turning the chill over. Fig. 3 represents any of the intermediate cross sections of Fig. 2 and also shows a section of a "hot refractory cover", 3, applied to the chill, 1, and a section of the ingot, 4, in the chill. The dotted lines in this figure represent planes of crystallization advancing from the heat absorbing walls of the chill. The final plane is almost flat and coincides with the surface of the ingot. The under side of this refractory cover, 3, is to be heated above the melting point of the steel being cast and applied immediately after the chill is filled so as to cause the surface below it to be the last of the metal to solidify.

In applying heat to the top of the ingot to delay the surface solidification I contemplate using any of the methods now practised in this art. I prefer the preheated cover since it has no chemical action on the metal if, as should be the practice, the chill is not filled clear to the top. The fact that the cover will lose heat will not prevent the desired effect since it is only intended that the surface solidification should be the last to occur and the effect of the cover is to furnish the necessary delay and to prevent any air chilling and consequent crusting over of the metal.

In the present practice the greater the length of the ingot for heavy work the greater the loss due to pipes and spongy tops. It results that thick ingots with an amount of rolling more than enough to develop the desired fiber in the finished product is the

common practice. In my process the ingot may be cast with a large ratio of length to its weight and no unnecessary rolling need be done on it. An approximately square ingot with a length of from eight to twelve times its thickness will crystallize more quickly and therefore with less "segregation" by my method than by the common practice.

In my method the chemical and physical variations, induced by the position of the chill and the consequent directions of cooling and crystallization, will occur transversely of the resulting ingot. All cross sections of the ingot will be alike since each one will contain its proportionate part of the top and bottom of the ingot.

Outside of the chills, heretofore described, the apparatus required for carrying out my improvement is not of any especial design. Furnaces for heating covers, if that method of heating the top of the ingot should be used, may be of any form that will heat the cover to the required degree.

Ingots cast horizontally are well known. Such ingots are subject to air chilling even when covered with carbonaceous material, which latter is put on at times primarily to prevent oxidation, and these latter crust over and trap the liberated gases with a loss of solidity in the ingot. My process requires the surface heat to be maintained at such a degree that crusting over of the top surface does not occur until the final solidification. Ingots have been cast horizontally in chills. Such ingots, being chilled on four long sides have no relief from the pipe that forms from the contraction of the heated central part after the outer shell has cooled enough to solidify. In this case a pipe forms in the upper longitudinal part of the ingot, the gases are trapped and the ingot is not solid.

In making chills for my process it is not necessary to use the particular design shown in the drawings. Those are shown merely to indicate the change in general effect required by my process. Chills for my process may be made by any construction now practised in this art when due consideration is given to the change of conditions under which the chill is used. The thickness of metal in the chill and the amount of draft required to readily release the ingot are easily adaptable from the present art.

I claim:

1. The process of forming an elongated ingot by pouring molten steel into an elongated horizontal chill, adapted to chill the bottom and both sides of the resulting ingot, and the immediate application by means of a hot gaseous envelop of sufficient heat to the surface of the metal just poured to cause said surface to be the last of the metal to solidify and to permit the escape of gases being expelled from the steel.
2. The process of forming steel ingots

which process comprises pouring the steel into shallow molds; then controlling the temperature of the poured steel by radiant heat whereby the isothermal zone of fusion measured at a mid transverse cross-section of the mass gradually advances inwardly and upwardly from coincidence with the surfaces of the mold to coincidence with the top surface of the steel mass.

10 3. The process of forming steel ingots to eliminate defects in said ingot, which process comprises pouring molten steel to form a shallow pool of molten steel; then controlling the temperature of the steel by controlling the temperature of the gases over the steel in such manner that solidification proceeds gradually from the sides and bottom of said pool while the surface thereof is maintained fluid, until the top surface of 20 the ingot is the last portion thereof to solidify.

4. The method of forming steel ingots and the like, which method comprises forming the ingot on its side by pouring the molten steel into a shallow elongated mold; then controlling the temperature of the molten mass by radiant heat applied to the surface of the mass to cause the molten steel to gradually solidify from the bottom of 30 the ingot to the top in such manner that the isothermal zone of solidification gradually travels from the sides and bottom of the steel mass upwardly and inwardly with the maximum depth of molten steel maintained at the middle of the cross-section of the ingot and the zone of maximum heat maintained at the surface of the ingot so that the steel at the surface of the ingot is the last to solidify.

40 5. The method of forming steel ingots, which method comprises providing a mold having its maximum longitudinal direction substantially horizontal; then pouring molten steel into said mold; then applying heat by means of a hot gaseous atmosphere to the surface of said mold while allowing the bottom and side portions of said mold to cool, whereby the top surface of said mold is maintained liquid up until the moment 50 of total solidification of the metal, thereby permitting free escape of the gases being expelled from the steel.

6. The method of forming ingots of steel and the like, which method comprises providing a relatively long shallow mold; then pouring the molten metal into said mold; then controlling the temperature gradients in said metal by means of a hot gaseous envelop maintained over the metal in such 60 manner that the crystallization of the metal mass proceeds inwardly and upwardly from the side walls and bottom of the mold toward the top surface of the ingot so that gases expelled during the crystallization of 65 the metal escape from the metal mass by

rising upwardly through a shallow molten layer and over an area which substantially includes the maximum length of said ingot.

7. The process of forming steel ingots to produce an ingot of substantially uniform cross-section from one end to the other thereof, which process comprises pouring the steel into shallow molds; then controlling the temperature of the steel by maintaining a hot gaseous envelop over the surface of 70 the steel with the temperature control such that cooling of the metal mass proceeds gradually from the sides and bottom of said mass whereby gases expelled during solidification at all times may escape vertically 80 through molten metal and wherein metal at the surface of the mold is last to solidify.

8. The method of forming steel ingots and the like, which method comprises pouring the molten steel into a shallow elongated chill mold, then controlling the temperature of the molten steel by providing a hot gaseous envelop in contact with the surface of the steel to cause the solidification of the steel to occur along cupped zones 85 which gradually change in shape from substantially the form of the chill mold surfaces to that of the top surface of the ingot whereby vertical lines from any portion of the solidifying zone extend upwardly 95 through molten steel to the hot gaseous envelop.

9. The process of forming ingots of steel having substantially a uniform cross-section from one end to the other, which process comprises pouring the molten steel into a shallow elongated chill mold; then maintaining a hot gaseous envelop in contact with the surface of the steel to control the temperature of the steel whereby crystallization 100 of the ingot gradually proceeds from the bottom and sides of the ingot toward the top thereof in such manner that vertical lines from the zone of crystallization at all times pass through molten steel to the hot 110 gaseous envelop, whereby gases emitted during the crystallization process may escape into the hot gaseous envelop.

10. The method of forming steel ingots and the like, which method comprises molding the ingot on its side in a chill mold with the top of the mold open; then providing a hot gaseous envelop over the top surface of the ingot and controlling the temperature of the ingot whereby crystallization proceeds gradually from the sides and bottom of the mold upwardly in such manner that the angle of the side of the crystallizing zone gradually changes from the angle of the sides of the mold to the angle of the top 125 surface of the ingot and in such manner that a layer of molten steel at all times covers the crystallizing zone up until complete solidification has taken place.

11. The method of forming steel ingots 130

and the like, which method comprises casting the ingots in shallow chill molds; maintaining a hot gaseous envelop over the surface of the steel and controlling the cooling of said steel whereby the heat gradient at all times during solidification runs from the top surface of the steel to the bottom and side walls thereof, and the action of solidification moves from the bottom of the mold 10 to the top surface of the ingot.

12. An article of manufacture comprising an ingot of steel with the lines of iso-crystallization therein comprising cuffed zones extending lengthwise of said ingot 15 with the width of the mouth of the cups being substantially constant and with the maximum zone being substantially the shape of the sides and bottom of said ingot and the minimum zone being substantially coincident with the top side of the ingot.

13. An article of manufacture comprising an elongated ingot of steel molded in an open mold with the longest dimension of the mold being substantially horizontal and wherein the iso-crystallization of the metal 25 said steel comprises a plurality of zones extending lengthwise of the ingot and from the bottom side of said ingot to the top side thereof with the maximum zone being substantially coincident with the ends, side 30 walls, and bottom side of said ingot and the minimum zone being substantially coincident with the top of said ingot.

Signed at Los Angeles, California, this 11th day of August, 1917.

RAY G. COATES.

Witnesses:

W. V. MERWIN,  
H. S. ROLLINS.